

Aug. 23, 1932.

R. TANBERG

1,873,362

POROUS LIGHTNING ARRESTER

Filed Aug. 6, 1929



Fig. 1.



Fig. 2.



Fig. 3.

INVENTOR  
Ragnar Tanberg.

BY  
Chestley S. Barr  
ATTORNEY

## UNITED STATES PATENT OFFICE

RAGNAR TANBERG, OF PITTSBURGH, PENNSYLVANIA, ASSIGNOR TO WESTINGHOUSE ELECTRIC & MANUFACTURING COMPANY, A CORPORATION OF PENNSYLVANIA

## POROUS LIGHTNING ARRESTER

Application filed August 6, 1929. Serial No. 383,924.

My invention relates to lightning arresters, and more particularly to a laminated or striated form of arrester that operates on the porous-block principle, as described in a co-pending application of J. Slepian, C. E. Krause and myself, Serial No. 379,899, filed July 22, 1929, and assigned to the Westinghouse Electric & Manufacturing Company.

In this copending application, is described a lightning arrester in which a lightning discharge, in passing therethrough to the ground, is confined within the minute pores of porous insulating material, such as porcelain, brick, or the like, but more particularly as in composite material of kaolin clay and carborundum, that has been molded into the form of a disc and fired to obtain the desired mechanical strength. It has been found that, if an electrical discharge is confined to spaces of very small size, say less than 1 mil in diameter, and preferably of the order of  $10^{-2}$  mil, said spaces being bounded by walls of insulating material or leaky insulating material, the voltage necessary to maintain the discharge is substantially the same as the voltage required to cause the breakdown of the confined space; and that, as soon as the discharge has passed, there is a quick extinguishing or de-ionization of the arc that prevents the power current of the transmission line from following the lightning discharge to ground. Such an arrester, composed of a porous block, when applied to a transmission line, will limit very satisfactorily the over voltages of the line to safe values, by providing a discharge path to ground for any abnormal charges induced in the line by lightning phenomena.

One form of composite porous blocks which has been utilized with good results is a modification of the discs utilized in the well-known auto valve arresters, described in the Slepian Patent No. 1,509,493, which are composed of kaolin clay, carborundum and lampblack for giving them a resistivity of the order of  $10^2$  ohms per centimeter cube or from 1 to about 200 ohms per centimeter cube. In order to make these auto valve discs applicable to operation on the porous-block principle, they are heated to a high temperature for

oxidation of the lampblack to increase their resistance some  $10^4$  or  $10^5$  times. Such an oxidized disc,  $\frac{1}{8}$  inch in length or thickness by 3 square inches in cross section, has a very high resistance of the order of  $10^4$  to  $10^6$  ohms, preferably about 30,000 ohms per disc. Even though the increase in resistance is not to the extent that the material may be termed a perfect insulating material, it is of the order of a leaky insulator or semi-conducting.

By the provision of a slight conductivity along the surfaces of the pores, or in the walls of the pores, the breakdown potential through the pores of the material is reduced to a lower value without lowering the cutoff voltage of the material, or the voltage at which the discharge ceases and, at the same time, the current-carrying ability of the material is increased, with consequent increase in the life during repeated passing of discharges. A very favorable performance characteristic is obtained with such a disc, surpassing, to a great and noticeable degree, the performance of arresters prior thereto. The desired conductivity when using auto valve discs may be obtained by controlling the amount of oxidation.

Though discs which may be obtained by oxidizing are preferred, it should be understood that I may utilize any porous composite disc having the desired resistivity and other electrical characteristics. For instance, it has been found that discs made of varying proportions of carborundum and clay, but omitting the lampblack constituent, have proved very favorable. These latter discs, when made, are fired in graphite-lined furnaces and obtain their slight conductivity mainly from gaseous fumes inherent in graphite furnaces.

However, the size of the discs that can be practically manufactured can carry, without rupturing, currents less than those inherent in high-voltage transmission lines where application of this porous arrester, having the very favorable performance characteristic, is desired. Such arrester must stand currents of the order of 1000 amperes, and above, without rupturing. The natural thing to assume is that discs made of the same

composition of materials as the auto valve disc could be larger in size, particularly in area, but it is found that, when this is attempted, great difficulty is encountered in the manufacturing process, thereby providing a mechanically imperfect and weak disc. Besides, it is of importance to keep the dimensions of the arrester as small as possible.

The potential of the transmission lines to which the application of the arrester is desired is also many times higher than the potential which successfully can be withstood by a single porous disc of thickness suitable for practical manufacture.

It is the object of my invention to provide a lightning arrester, operating on the porous-block principle and made of composite material, which will stand currents of the order of 1000 amperes and upward and which is suitable for the protection of high-voltage transmission lines.

In practicing my invention, I stack a plurality of composite, high-resistance discs, one on top of another. I so treat the discs prior to stacking, with a solution of a conducting material, as to render the end surfaces, in which the conducting material has penetrated to something of the order of one-half or three-quarters of a millimeter, relatively highly conducting as compared to the bulk of the block. I thereby provide the effect of a graded resistance from the surface of the disc to the interior. The discs are then cemented together in a stack by a conducting cementitious material. The current, in passing through this stacked or laminated arrester, upon reaching a conducting region, is well distributed over the entire cross-section, thereby eliminating concentration of current which might cause puncture of a porous disc. To further improve the results, I cement a disc of relatively low-resistance, such as an auto valve disc to each end of the stack, as will be subsequently described. Such an arrester carries heavy surge currents over 1000 amperes without failure and, in doing so, gives the desired characteristic. At the same time it can be made suitable for any line voltage by cementing the proper number of discs together.

For a better understanding of my invention, reference may be had to the following description, taken in connection with the accompanying drawing, in which;

Figure 1 is a sectional view of my striated or laminated porous-block lightning arrester element, with a diagrammatic showing of the line connections.

Fig. 2 is a curve diagram showing the performance characteristic of one of my laminated arresters having a maximum current rating of the order of 1000 amperes, and

Fig. 3 is a curve diagram showing how the potential characteristic of a given porous

arrester disc is influenced by varying the resistance.

In Fig. 1, my invention is illustrated in a laminated arrester element of a size capable of protecting a transmission line with 2300 volts (R. M. S.) to ground. In making my laminated arrester, I utilize a plurality of high-resistance porous discs, 1a, 1b and 1c, the resistivity of each of said discs being from  $\frac{1}{2}$  megohm to 10 megohms per centimeter cube, and the number of said high-resistance discs depending upon the potential rating of the system to be protected as will hereinafter appear. My laminated arrester has end discs 2a and 2b of relatively low resistance, only one being shown on each end, but a plurality might be used of different resistance to provide a graded resistance, the resistivity of these discs being of the order of a few ohms per disc, or of the order of  $10^2$  ohms per centimeter cube.

The several high and low-resistance discs are held together by conducting cement layers 3 for solidly holding the discs in stacked relation and, at the same time, providing conductivity over the surfaces of the discs in order to effect an equal distribution of current and, in this way to make it possible for the discs to pass heavy surge currents without being punctured or destroyed.

Metallic contact plates 4a and 4b are disposed on each end of the stack to serve to equalize the distribution of the current, as well as to provide a good contacting surface. In addition to the metal plates, it is preferable that the low-resistance end discs 2a and 2b shall have a copper-plated contact surface for engagement with the metallic plates 4a and 4b.

In order to prevent flashover of the discs along the edges, I coat the periphery of the integral stack with some insulating material. For example, shellac provides a good insulation and does not crack.

I preferably treat the high-resistance discs 1a, 1b and 1c, in order to provide them with the thin, highly conducting surface layer previously mentioned, and, for this purpose, I prefer to utilize a thin water-glass solution having mixed with it a large quantity of powdered conducting particles, such as lampblack. I allow the discs to soak in this solution for about an hour, which is sufficient time for the solution to penetrate into the discs to a distance of one half of a millimeter or thereabouts, filling the pores, near the surfaces of the discs, with conducting lampblack, and giving each of the discs a conducting surface, whereby good distribution of current is obtained. At the same time, the rating of the disc is not lowered because the penetration of the conducting solution is so very small, as compared with the total disc-thickness of  $\frac{1}{8}$  inch or about 3 millimeters.

For cementing the discs together, I also

utilize a mixture of liquid water-glass and lampblack, but one which is thicker or less diluted. This cement layer 3 provides additional conductivity between adjacent discs, and hence it also aids in securing the desired distribution of current over the entire cross-section of each of the discs or lamination of my laminated arrester.

After the discs are stacked, any superfluous water-glass solution, that may be left on the edges of the discs, may be washed off with water. Since the impregnation is so slight, it is found that ordinary washing with water is sufficient, but, in addition, if desired, the edges may be ground on a stone. The assembled discs are then allowed to dry for about six hours at 70° C. and thereafter baked for about six hours at 150° C.

Although I have only mentioned water glass and carbon, I find that solutions or suspensions of almost any other conducting liquid may be utilized with a fair degree of success.

As stated above, the discs themselves are of composite material and may be made from the relatively low-resistance auto valve discs described in the above-mentioned Slepian patent. These auto valve discs have an initial resistance of the order of two ohms, for a cross section of 3 square inches and a length of  $\frac{1}{8}$  inch. They are heated sufficiently to burn out or oxidize most of the lampblack, leaving but a small amount in the discs and preferably just enough to ensure satisfactory action of a porous arrester, the resistance of each disc being increased to something of the order of 30,000 ohms. These treated discs have fine pores, having an average diameter of about .03 mil, and have a resistivity of something of the order of 2 megohms per centimeter cube.

The incorporation of a small trace of conducting material in a porous-block arrester has been found to have two very important effects, which may very probably be explainable as follows. The addition of conducting material has the effect of lowering the breakdown potential without appreciably changing the cutoff potential, thereby improving the characteristic of the arrester considerably. The addition of the conducting material has also the effect of flattening out the voltage-current characteristic of the arrester, by making the breakdown voltages of the pores, more nearly equal, thereby also causing the discharge to be distributed over a larger number of pores which will increase the life and current-carrying ability of the arrester.

The manner in which these two results are effected may very probably be explained somewhat as follows. For a given length of pore, in an insulating material, the breakdown voltage is effected but very slightly by the size or diameter of the pore, but the volt-

age gradient of the discharge in the pore, once break-down has occurred, increases very rapidly as the diameter of the pore is decreased or, conversely, the arcing voltage or maintaining voltage or cut-off voltage is very much lower for large pores than for small pores. In any natural or inherently porous material, there are some slight irregularities in the lengths of the various porous paths from one surface to another, so that the break-down voltages of all of the pores, in an insulating material, are not the same.

The effect of the slight traces of conducting material, which incorporated into the porous-block arrester material, is to produce extremely attenuated chains or needles of conducting particles disposed in the walls of the pores, so that the potential gradient or electrostatic field, in the pores between the opposite terminals of the arrester, is rendered non-uniform. These needles are believed to produce needle discharges which initiate the ionization of the gaseous material in the pores, thereby lowering the breakdown voltage and making the breakdown voltages of all of the porous paths more nearly equal. In other words, the effect of the needle discharge is more noticeable in the porous paths of high breakdown voltage than in those having the lower breakdown voltages. The cross-sections of these needles or chains of minute conducting particles, probably making loose contacts with each other, are so small that no material current can be carried by the needles, so that, when the discharge is once initiated, by breaking down the gaseous space by reason of the ionization produced by the needle discharges, the discharge current is distributed throughout the entire volume of the pores without being affected by the presence of the needles, because the current carried by the needles is wholly negligible, as compared with the current carried by the pores.

This explanation, which seems to be the proper explanation of the phenomena involved, also explains the fact that a larger quantity of conducting material is required for porous arresters having large pores than for the more finely porous materials, because the voltage gradient necessary to maintain an arc in a large pore is much smaller than in a small pore, so that more conducting material must be utilized, in the case of the large pore, in order to bring down the breakdown voltage sufficiently close to the maintaining or cut-off voltage. Preferably, only enough conducting material is added, for any type of porous-block arrester, to bring down the breakdown voltage to the vicinity of the cut-off voltage. Too much conducting material will needlessly increase the leakage loss, which is measured in milli-amperes, or fractions of milli-amperes and, as the quantity of conducting material is increased more

and more until it becomes excessive, it will begin to short-circuit the arcing paths through the pores because the voltage drop in the conducting paths will become smaller than the minimum voltage drop necessary to maintain the arcs in the small pores.

In general, therefore, the desirable or permissible resistivity of the porous-block arrester material depends upon the fineness of the pores. Nevertheless, the resistivity of the porous-arrester material is always so high that it is of the order of the resistivity of a leaky insulator, being measurable in units of the order of  $10^{-6}$  or  $10^{-7}$  ohms per centimeter cube, as against something like 100 ohms for the auto valve arrester disc,  $10^{-3}$  ohm for carbon, and  $10^{-6}$  ohm for copper. A wide range of diameters of the pores seems to be available, ranging probably, anywhere from a diameter of the order of 1 mil, or possibly more, to diameters of the order of  $10^{-3}$  mils, or possibly less. These values are not absolute and sharply fixed, as desirable results may be obtained with a ten-fold or even a hundred-fold departure from any of the values stated.

In Fig. 3, is shown the manner in which the cut-off voltage changes, with variations in the resistance of discs having a diameter of 2 inches, a length or thickness of  $\frac{1}{8}$  inch, and pore-diameters of about .03 mil. For resistances up to about 35,000 ohms per disc, the curve takes the form of an approximately straight line, having a slope of approximately 40 volts per thousand ohms. At about the 35 thousand-ohm point, the curve begins to straighten out, so that there is no material advantage in utilizing materials of much higher resistance. With this resistance of 35 thousand ohms per disc, or about 2 megohms per centimeter cube, good current-carrying ability is ensured. A single disc has a cut-off voltage of 1600 volts, as may be seen from the curve in Fig. 3. A single disc, without means for ensuring good distribution of the discharge, will discharge a momentary current of the order of 60 amperes, but probably could not pass more current without becoming impaired or punctured.

By stacking the high-resistance discs just described, and providing for good distribution of current at the surfaces of the discs, I obtain a characteristic, such as shown in Fig. 2. Discs so stacked will carry current of the order of 1000 amperes. A stack utilizing three high-resistance discs, as shown in Fig. 1, including the relatively low-resistance end discs, gives a maximum voltage of about 12,000 volts, and a cut-off voltage of about 3800 volts crest value. Such an element is capable of protecting a transmission line having a root-mean-square voltage of 2300 volts from line to ground. To provide an arrester for higher-voltage systems, a larger number of high-resistance discs may be utilized or several elements may be stacked.

As is usual in arresters of this type, my arrester is preferably provided with a series gap device 10, as indicated in Fig. 1.

The term cut-off voltage or cut-off potential, as used in my description denotes the lowest voltage that will maintain the arc discharge through the pores of the semi-conducting material.

I claim as my invention:

1. A striated porous-block arrester having a plurality of porous discharge discs stacked and cemented together with conducting cement, said discs being made of semi-conducting porous material operating on the principle of discharges through the pores, said pores being so fine that the voltage-gradient necessary to maintain a discharge is measured in thousands of volts per inch, and the amount of conducting matter in said porous material being barely sufficient to bring the breakdown voltage substantially down to the cutoff voltage in each of the pores carrying current. 75

2. A laminated porous-block arrester having a central portion of semi-conducting porous material operating on the principle of discharges through the pores, said pores being so fine that the voltage-gradient necessary to maintain a discharge is measured in thousands of volts per inch, and the amount of 90 conducting matter in said porous material being barely sufficient to bring the breakdown voltage substantially down to the cutoff voltage in each of the pores carrying current, said arrester having top and bottom terminal portions, each of said terminal portions having a plurality of layers of conducting material of progressively increasing conductivity, starting with an inner layer disposed next to the said central portion and having more conductivity than said central portion, and including a metallic end terminal plate. 95

3. A laminated porous-block arrester having a central portion of semi-conducting porous material operated on the principle of discharges through the pores, said pores being so fine that the voltage-gradient necessary to maintain a discharge is measured in thousands of volts per inch, and the amount of 110 conducting matter in said porous material being barely sufficient to bring the breakdown voltage substantially down to the cutoff voltage in each of the pores carrying current, said arrester having top and bottom terminal portions, each of said terminal portions having a plurality of layers of conducting material or progressively increasing conductivity, starting with an inner layer disposed next to the said central portion and having more conductivity than said central portion, 115 and including a metallic end terminal plate, the said layers and central portion being all cemented together into a single solid body. 120

4. In the manufacture of porous-disc lightning arresters the method which comprises 125

soaking semi-conducting porous discs in a conducting solution, providing a layer of relatively high conducting cement on the end surfaces of the discs, stacking said discs together, drying and baking the assembled structure.

In testimony whereof, I have hereunto subscribed my name this 30th day of July, 1929.

RAGNAR TANBERG.

10

15

20

25

30

35

40

45

50

55

60

65